

Aug. 22, 1944.

P. G. DEUCHLER

2,356,570

COVERING ELEMENT

Filed Dec. 26, 1940



INVENTOR  
BY PHILIP G. DEUCHLER  
Alfred F. Ernst  
ATTORNEY

## UNITED STATES PATENT OFFICE

2,356,570

## COVERING ELEMENT

Philip G. Deuchler, Snyder, N. Y., assignor to Certain-Teed Products Corporation, New York, N. Y., a corporation of Maryland

Application December 26, 1949, Serial No. 371,799

4 Claims. (Cl. 117—5)

This invention relates to composition covering elements and to processes of making the same. More particularly the invention is directed to the production of thick butt elements of the felt base type which are coated with waterproofing adhesive material and which carry a surfacing of comminuted material embedded in the coating. The element may have an edge of the body thereof divided by slots to form a plurality of tabs and if desired the surfacing carried on the body of the element may be of contrasting appearance to that upon the tab portions.

Thick butt shingles have been produced by providing a base element with a thicker adhesive coating on the butt or tab portion of the element than upon the body portion thereof. Tapered shingles have also been produced by providing the base element with a coating which is of gradually decreasing thickness from the butt edge of the element.

Variation in thickness of the coating on the face of the element has been obtained by applying over the entire face of the element a relatively thick adhesive coating and then doctoring or scraping away portions of the coating so as to reduce the thickness thereof on the body portions of the element relative to the tab or butt portions.

Another method by which variation of the thickness of coating on the base element has been secured is by the application of separate coatings of different thickness directly upon different portions of the face of the base element. In all such elements the coatings may be surfaced with comminuted material of the same or contrasting character upon the body and tab portions of the element.

When contrasting comminuted materials are applied to different portions of the coating on the base element, in carrying out the surfacing operation difficulties have been encountered in securing a sharp line of demarcation between the contrasting areas. This condition may be caused in some cases by the bounce of granules applied to one area, as the granules strike the sheet, across an intended line of demarcation to the adhesive coating to fall upon an adjacent contrasting color area. Spread of the granules to the adjacent area may also be caused by the rolling action of the granules as pressure is applied to embed them in the coating. Unintended delivery of granules to the adjacent area also may be caused by irregularity of flow of the granules fed to the sheet. When the contrasting comminuted material is subsequently ap-

plied to the portion of the coating which it is intended to surface, it is prevented from adhering to the portions accidentally surfaced with the first granules and can adhere only to the 5 portion of the coating not surfaced accidentally or otherwise by these first applied granules. Intermixture and interplacement of the contrasting materials at or near the intended line of demarcation therefore results.

10 A similar unsatisfactory result frequently is obtained if the contrasting surfacing materials are applied simultaneously to the different portions of coating on the element because intermixture of the granules of contrasting character 15 may occur adjacent the common boundary as they move toward the coating upon the sheet. In some instances merging of the contrasting surfacing materials at their common boundary may not be objectionable or may even be considered desirable. However, such merging of 20 color areas is particularly objectionable in the production of sidings which are intended to simulate brick units laid up in mortar. In manufacture of brick simulating siding it is essential that a clean, sharp line of demarcation be 25 secured between the brick and mortar areas so that a satisfactory representation of brickwork may be effected.

A prior art method of producing thick butt 30 elements by which a sharp line of demarcation between the contrasting areas may be secured is the so-called "overlay" process. In the "overlay" process the entire surface of the base element is coated with adhesive material 35 and comminuted surfacing material is then applied to the entire coated face and partially embedded in the coating. A second or overlay coating of adhesive material is applied to the surfacing material on the portions of the element 40 intended to be of contrasting appearance to said first surfacing and a second surfacing of a character contrasting to said first surfacing is applied to the second or overlay coating and partially embedded therein.

45 Siding which effectively simulates brickwork may be produced by the "overlay" process because a sharp line of demarcation can be obtained when the second coating is applied to portions of the first or mortar color surfacing 50 and thereafter surfaced with brick color comminuted material. However, the comminuted material first applied to the areas which are subsequently covered by the overlay coating is wasted so far as the appearance and weather protection of the finished product are concerned.

The present invention is directed to a new method of producing thick butt covering elements which is efficient and economical to carry out.

Another object of this invention is to provide a covering material or an element having areas contrasting in appearance sharply demarcated from each other at their common boundary without the disadvantages of the overlay process.

The movement of my invention may be practiced by applying to a base sheet of suitable material a coating of adhesive material so as to cover an entire surface of the sheet. I next apply a comminuted surfacing material to the coating on a limited area of the sheet to leave unsurfaced a portion of said coated sheet. The surfacing is partially embedded in the coating and the excess thereof is removed.

As brought out above, the boundary of the surfaced area may not be sharply demarcated from the area intended to be unsurfaced because of bounce of the surfacing over the intended line of demarcation or its uncontrolled delivery to the portion of the coating desired to be kept free of the first applied surfacing material.

I next apply a second coating of adhesive material directly to the area left bare of the first surfacing so as to be superposed upon the first coating and become adhesively bonded thereto. I apply this superposed coating so as to cover the accidental marginal deposit of surfacing material on the first coating across the intended line of demarcation upon the area intended to be free of said surfacing. I so apply this second coating that a sharp boundary line of coating is formed where it meets the previously surfaced area. This second coating may effectively increase the thickness of the portions of the sheet to which it is applied.

The second or superposed coating is then surfaced with comminuted material contrasting in character to the first applied surfacing material which second surfacing is partially embedded into the superposed coating.

In the product of my invention there is not wasted a substantial quantity of granular surfacing material under the second coating as in the product of the "overlay" method but there is provided instead an area comprising two coatings bonded together over the portion of the covering desired to be thickened without the presence of an intermediate layer of granules between the coatings.

Fig. 1 shows an assembly of the siding elements of the invention.

Figs. 2, 3 and 4 show the progressive steps in carrying out the method of the invention, Fig. 4 being a section taken on the line 4-4 of Fig. 1.

Fig. 5 is an enlarged section of the butt portion of the element of Fig. 4.

Fig. 6 illustrates the steps in the production of the elements of the invention by a continuous process.

Fig. 7 is a modification of the element shown in section in Fig. 4.

Fig. 8 is a further modification of the element shown in section in Fig. 4.

In the assembly of siding elements shown in Fig. 1, each of the elements 1 comprises a mortar simulating area 10 and a plurality of brick simulating areas 9 separated by slots 7.

The body portion of each of the elements in the area 10 thereof carries a surfacing 4 which may be comminuted mineral material, such as slate granules of mortar color. The areas 9 of

the tab portion carry a surfacing 6 of brick color which extends from the butt edge of the element a distance to represent the depth of a brick.

5 A plurality of slots 7 extend from the butt edge of the element a distance equivalent to the thickness of a brick plus the width of a mortar joint. The slots 7 are equivalent in width to the usual vertical mortar joint and are spaced apart along the butt edge of the element a distance equivalent to the length of the bricks. As a result of the arrangement of the slots a plurality of tabs 8 having brick areas 9 along the butts thereof and between slots 7 are produced on the portion of the element to be exposed to the weather.

10 The siding elements 1 are assembled with the butt edges of the tabs 8 matched to the inner ends of the cut-out slots 7 of the element in the underlying course and arranged with the slots of the successive courses staggered or off-set in order to provide an effective simulation of brick units laid in mortar.

20 Figs. 2, 3 and 4 show steps of a process by which the siding elements 1 of Fig. 1 may be produced.

25 A base element 2 which may be of felted fibrous material saturated with a waterproofing material, such as asphalt, is shown in the figures with a coating 3 of adhesive material thereon, such as asphalt which has been applied in heated condition uniformly over a face thereof.

30 On the area of the body portion of the base 2 I apply to coating 3 a surfacing 4 of granular material, such as mineral granules, of suitable mortar color, so as to leave unsurfaced an area of coating 3 the thickness or depth of a brick unit. The area 10 thus is spaced from the butt edge of the element approximately the depth of the brick area. I partially embed the granules 4 into the coating 3 and thereafter remove the excess granules from the surface of the element.

35 In commercial practice it is extremely difficult to control the application of the surfacing 4 on the coating 3 so that only a defined area 10 will be surfaced therewith because some of the granules such as those indicated at 44 will bounce across the intended line of demarcation or otherwise become deposited on and partially embedded in the portion of the coating 3 desired to be left bare of mortar color surfacing material 4.

40 I next apply a layer of adhesive coating 5 which may be heated asphalt of the same or different character as the coating 3. The coating 5 may be printed directly upon the unsurfaced portion of coating 3 so as to extend from the butt edge of the element 2 across the width of the tabs a distance equivalent to the depth of a brick unit such as 9. Any accidental deposit of mortar color granules 44 on the coating 3 beside the area 10 will therefore be covered by the superposed coating 5 which becomes united with the coating 3 lying theretherein.

45 To the adhesive coating 5 I then apply a surfacing of comminuted material 6, which may be brick color granules, and partially embed the granules 6 into the coating 5 so as to bond them thereto. I then remove the excess granular surfacing 6 from the surface of the element.

50 Limitation of the brick color granules 6 to the superposed coating 5 need not be attempted because even if the surfacing 6 were to bounce or accidentally become deposited across the line of demarcation it would not become secured to the mortar area 10 because the coating 3 on the mortar area 10 has been rendered non-adhesive by the application of the surfacing 4 thereto. A

clear cut line of demarcation therefore can be obtained between the surfacing materials 4 and 6 on the respective mortar area 10 and brick areas 9.

Fig. 6 illustrates how the invention may be carried out to produce siding units in a continuous manner. It will be noted that the zones II, III and IV of Fig. 6 correspond to the sections of the element 1 of Figs. 2, 3 and 4.

A sheet or web of fibrous felted material 12, in the particular embodiment shown of a width equivalent to the transverse to the course width of three elements and of indefinite length, is carried through a roofing machine in the usual manner.

The portion of the felted web 12 in zone I has been previously saturated with asphalt and carries a coating of asphalt 13 in heated condition applied uniformly on the surface thereof. The web is then carried to suitable surfacing devices where the longitudinal bands of surfacing 14 of mortar color granules are applied to the coating 13 on the portions of the web intended to be the mortar areas 10 in the finished element. As can be seen in zone II of Fig. 6, the granules of surfacing 14 although intended to form a sharp line of demarcation with the unsurfaced areas of coating 13 may bounce or otherwise be carried over the intended line of demarcation and adhere to the adhesive coating on the other side of said line of demarcation as indicated by the granules 144. The surfacing 14 is partially embedded in the coating 13 and the excess thereof removed from the surface of the web.

I next apply in zone III by suitable means such as a print roll the bands of adhesive coating 15 directly upon the portions of the web carrying the still unsurfaced coating 13 so as to form a sharp line of demarcation where the coating 15 and surfacing 14 meet.

The coating 15 is applied so that the surfacing 14 becomes covered by the coating 15. I preferably slightly overlap the marginal portions of the surfacing 14 with the coating 15 so that meeting of the coating 15 and the surfacing 14 as well as the covering of the granules 144 by the coating 15 is assured even though weaving of the web from side to side occurs as it passes through the machine. Sufficient marginal overlap of the surfacing 14 by the coating 15 may be provided in order to compensate for the greatest amount of side to side movement or weave of the web likely to occur as it is being carried through the print rolls for printing coating 15 on the sheet.

As illustrated in zone IV of Fig. 6 the superposed coating 15 is surfaced with brick colored granules 16 and this surfacing is partially embedded in the coating 15 and the excess thereof removed.

The surfaced web is then fed to suitable cutting apparatus which cuts out the slots 17 and separates the web along the dotted lines to produce the finished siding elements.

Within the scope of the invention the superposed coatings 5 or 15 may be of the same thickness as the underlying coatings 3 or 13 respectively or may be of greater or less thickness, dependent upon the effect desired.

By the use of asphalt coatings, having a high content of inert or mineral filler, I may apply coatings of substantially greater thickness than would successfully be applied before the development and use of such filled asphalt coating materials in the roofing industry. Such filled

coating may comprise blown asphalt having incorporated therewith about 30 to 60% by weight of fine inert filler material, as for example, ground dolomite limestone, talc, or slate flour.

5 In Figs. 7 and 8 I have shown sections which illustrate modified forms which my invention may take when two printed coatings are applied to the portion of the element to be exposed in order to secure a thicker butt section.

10 The element shown in Fig. 7 may be constructed by utilizing the coated and partially surfaced base 2 as shown and described in connection with Fig. 2. I apply the adhesive coating 25, such as asphalt in heated condition, corresponding to the coating 5 shown in Fig. 4 so as to cover any accidental deposit of granules such as those shown at 44 on the portion of the element to be thickened. However in this modification I superpose upon the coating 25 another asphalt coating 27 15 into which comminuted material 6 may be partially embedded.

20 In Fig. 8 I have shown a further modification of my invention by which a sharp line of demarcation may be secured at the common boundary of contrasting surfacing material.

25 In the modification shown in Fig. 8 the coating corresponding to the coating 3 of Fig. 4 is made up of two separate portions 23 and 25 applied upon separate areas of the base 2 so as to 30 form contiguous coatings on the base 2. As illustrated in Fig. 8 the base 2 has an adhesive coating 23, such as asphalt in heated condition, on a face thereof so limited in extent as to leave an area of the base 2 bare of coating material 23.

35 To the coating 23 I apply comminuted surfacing material 4 of suitable appearance, partially embed the same in the coating 23 and remove the excess thereof from the face of the base. I then print an asphalt coating 25 directly upon the 40 portions of the base left bare of the coating 23 so as to be contiguous with coating 23 and superpose upon coating 25 another coating 27 of suitable adhesive material, such as heated asphalt, so that as to be bonded thereto. I then apply 45 comminuted surfacing material 6 to the coating 27 and partially embed the same therein.

50 If the embodiments of the invention shown in Figs. 7 and 8, are produced in a continuous manner similar to that shown in Fig. 6, I may provide for marginal overlap of the surfacing 4 by the coating 27 as described in connection with Fig. 6 in order to assure meeting of the coating 27 and surfacing 4 regardless of the weave of the sheet as it passes through the machine.

55 In practicing the above described methods of the invention it may be necessary with some coating materials to allow the first applied adhesive coating to partially or wholly set before a second adhesive coating is superposed directly

60 thereon. When asphalt coating, either filled or unfilled, is applied in heated condition to the base it is usually necessary to allow or cause the first applied coating partially to cool or congeal before a second coating of hot asphalt is superposed thereon in order that the two coatings may not merge or run, and thus fail to secure limitation of the printed coating to the areas intended to be covered thereby.

65 It is to be understood that the foregoing description is merely illustrative of the forms which my invention may take. I do not wish the scope of my invention to be limited to the examples discussed above. For instance, in the element 1 as shown in Fig. 1, I may omit the slots 7 and use 70 75 as a base merely a slab having uncut edges. The

surfacing 4 which simulates the mortar color in this case may be carried on the areas occupied by the slots 7 in the former embodiment as well as on the area 10. The coating 5 may be then printed upon the base to represent individual brick units spaced apart along the edge of the element.

My invention is not limited to siding elements simulating brick construction but may be utilized with any covering material to secure a sharp line of demarcation between contrasting color areas on a base in an efficient manner.

Having thus described my invention, I now claim:

1. A thick butt covering element for laying in courses in overlapping arrangement comprising a base sheet, a coating of asphaltic adhesive material in set condition covering a face of said base sheet, a surfacing of comminuted material bonded to and covering a portion of said coating of substantial extent on said face but leaving bare of said comminuted material an adjacent portion of said coating of substantial extent on said face, said portions meeting along a common boundary extending coursewise of said element, a second coating of asphaltic adhesive material in set condition superposed directly upon said bare portion of said first coating and adhesively bonded thereto and overlapping and interlocking with said comminuted surfacing on said first coating only slightly along a narrow portion at said boundary thereof which meets said bare portion, said second coating having bonded thereto comminuted surfacing material contrasting in appearance to said comminuted surfacing material which is bonded to said first coating.

2. A thick butt covering element for laying in courses in overlapping arrangement comprising a base sheet of generally rectangular shape having tabs separated by slots in said base extending inwardly from the coursewise edge of said element which is exposed in said arrangement for a substantial distance to form tabs of substantial area, a coating of asphaltic adhesive upon and extending fully over a face of said base, a surfacing of comminuted material bonded to and covering the portion of said coating which extends from a coursewise line adjacent the inner ends of said slots to the edge of the element remote from said coursewise edge but leaving bare the portion of said coating between said coursewise line and said exposed coursewise edge, a second coating of asphaltic adhesive material in set condition superposed directly upon said bare portion of said first coating and adhesively bonded thereto and overlapping and interlocking with said comminuted surfacing ma-

terial on said first coating only slightly along a narrow portion at said coursewise line, said second coating having bonded thereto comminuted surfacing material contrasting in appearance to said comminuted surfacing material which is bonded to said first coating.

3. Process of producing a thick butt covering element for laying in courses in overlapping arrangement which comprises applying to a base sheet a coating of asphaltic adhesive fully to cover the face of said element, applying to the portion of the area of said coating which is spaced from that coursewise edge of said element which is exposed in said arrangement a surfacing of comminuted material so as to be bonded to said coating but leaving bare the adjacent portion of the area of said coating which extends between said surfaced portion and said coursewise edge of said element, said portions both being of substantial extent in the direction transverse to said coursewise direction measured from the boundary therebetween, applying a second coating of asphaltic adhesive upon and directly bonded to said bare portion of said first coating and overlapping and interlocking with said comminuted surfacing material on said first coating only slightly along a narrow portion at said boundary, and applying to said second coating a comminuted surfacing material of contrasting appearance to said comminuted surfacing material which is bonded to said first coating.

4. A process of producing a thick butt covering element which comprises applying to an elongated base sheet a coating of asphaltic adhesive substantially completely to cover said base sheet, applying to bands of substantial width extending lengthwise of said sheet and spaced apart substantial distances widthwise of said sheet comminuted surfacing material so as to bond to said coating and so as to leave bare said space between said bands, applying to said spaces left bare of comminuted surfacing material superposed layers of coating of asphaltic adhesive extending lengthwise of said sheet between said surfaced bands and overlapping and interlocking with said comminuted surface material on each adjacent band only slightly along a narrow portion at the boundary between said surfaced bands and said spaces left bare of comminuted material, applying to said superposed layers of coating comminuted surfacing material contrasting with said first comminuted surfacing material, and cutting said sheets into covering elements with the portions thereof which carry said superposed layer of coating forming the thick butt portions of said elements.

PHILIP G. DEUCHLER.

CERTIFICATE OF CORRECTION.

Patent No. 2,356,570.

August 22, 1944.

PHILIP G. DEUCHLER.

It is hereby certified that error appears in the printed specification of the above numbered patent requiring correction as follows: Page 2, first column, line 10, for the word "movement" read --improvement--; and that the said Letters Patent should be read with this correction therein that the same may conform to the record of the case in the Patent Office.

Signed and sealed this 7th day of November, A. D. 1944.

Leslie Frazer

(Seal)

Acting Commissioner of Patents.